

1

3,150,093

## LUBRICANT COMPOSITION

Daniel B. Eickemeyer, Park Forest, Ill., and James E. Engelking, St. Paul, Minn., assignors, by mesne assignments, to Sinclair Research, Inc., New York, N.Y., a corporation of Delaware

No Drawing. Filed June 9, 1960, Ser. No. 34,892

4 Claims. (Cl. 252—46.3)

This invention relates to ester-based lubricant compositions containing a novel combination of additive agents. More particularly the present invention relates to ester-based lubricant compositions which exhibit increased oxidation resistance.

Organic compounds, such as lubricating oils, undergo oxidation upon exposure to air. This process is accentuated by elevated temperatures such as occur in engines and other operating machinery. When such organic compositions are used as motor or machinery lubricants, their stability is still further drastically reduced due to their contact with metal surfaces which give up metallic particles into the lubricant. Such abraded or dissolved metals or metal salts appear to act as oxidation catalysts in the lubricant causing the formation of primary oxidation products which in turn cause further degradation of the organic compounds present in the composition. In addition, water also causes corrosion of metallic surfaces and accentuates oxidation of the lubricant. Problems of this nature are encountered in mineral oils but appear to be particularly troublesome in synthetic oleaginous fluids exemplified by esters. These synthetic fluids are not sufficiently resistant to oxidation to be useful alone. They can, however, be adequately protected by use of small amounts of additives. Phenothiazine has been employed extensively to protect synthetic fluids against oxidation. Its activity, however, is not great enough to protect fluids for long periods of time above about 400° F.

It is the particular object of the present invention to provide an ester oil of lubricating viscosity that exhibits increased resistance to oxidation. Further, the additives of the present invention have proven far more effective than the conventional use of phenothiazine alone in reducing oxidation in synthetic ester fluids.

The present invention provides an improved ester-based lubricant composition containing minor amounts effective to retard oxidation, of phenothiazine, 5-alkyl-10,10-diphenylphenazasiline wherein the alkyl group is a lower alkyl group, i.e. generally of about 1-4 carbon atoms, preferably 2 carbon atoms and a compound selected from the group consisting of aminoquinoline, aminopyridine and their mixtures.

The rings of the siline compound may be substituted as for instance with alkyl groups. The additives of the present invention are added in amounts that provide a final ester-based synthetic lubricant composition exhibiting increased resistance to oxidation under temperatures such as in excess of 400° F. The amounts added should be soluble in the base oil into which they are introduced and these amounts will vary with the particular base oil utilized.

The preferred aminoquinolines for use in the present invention are 3-aminoquinoline and 8-aminoquinoline and their ring substituted derivatives, e.g. alkyl-substituted. Among the useful aminopyridines are 2-aminopyridine and the ring-substituted, e.g. alkyl substituted, aminopyridines. The aminoquinoline or aminopyridine may be added in amounts from about .01-5% by weight of final composition with a preferred amount of from about 0.1 to 2% by weight of final composition. The aminoquinoline or aminopyridine and the 5-alkyl-10,10-diphenylphenazasiline additive are normally added to the ester-

2

based by lubricant along the phenothiazine. The phenothiazine is usually present in amounts from about .01-5% by weight of the final composition with a preferred amount being from about 0.1-2% and the phenothiazine may be substituted as with alkyl groups, for instance on the nitrogen or in positions ortho and meta to the nitrogen. The 5-alkyl-10,10-diphenylphenazasiline component is generally added in amounts of about .01-5% by weight of the final composition with a preferred amount of from about 0.1 to 2% by weight of final composition. As aforementioned, the preferred diphenylphenazasiline component is 5-ethyl-10,10-diphenylphenazasiline. For obtaining best results, the relative concentrations of the additives may vary with the particular ester lubricant employed and may also be dependent upon the characteristics of the final lubricant composition desired. Normally it is preferred that at least about 1 part of 5-alkyl-10,10-diphenylphenazasiline and at least about 0.5 part of aminoquinoline or aminopyridine to one part of phenothiazine be utilized, e.g. about 1-2.5 parts 5-alkyl-10,10-diphenylphenazasiline and about 0.5-1.5 aminoquinoline or aminopyridine to one part of phenothiazine. Increasing the amounts of 5-alkyl-10,10-diphenylphenazasiline and aminoquinoline or aminopyridine will generally be desired.

The lubricant composition of this invention includes as the major compound a base oil which is an ester of lubricating viscosity which may be, for instance, a simple ester or compounds having multiple ester groupings such as complex esters, polyesters, or diesters. These esters are made from mono- and polyhydroxy aliphatic alcohols and aliphatic carboxylic acids, frequently of about 4 to 12 carbon atoms; aliphatic including cycloaliphatic. The reaction product of a monohydroxy alcohol and a monocarboxylic acid is usually considered to be a simple ester. A diester is usually considered to be the reaction product of 1 mole of a carboxylic acid, say of 6 to 10 carbon atoms, with 2 moles of a monohydric alcohol or of 1 mole of a glycol of 4 to 10 carbon atoms with 2 moles of a monocarboxylic acid of 4 to 10 carbon atoms. The diesters frequently contain from about 20 to 40 carbon atoms. One complex ester is of the type X-Y-Z-Y-X in which X represents a monohydric alcohol residue, Y represents a dicarboxylic acid residue and Z represents a glycol residue and the linkages are ester linkages. Those esters, wherein X represents a monoacid residue, Y represents a glycol residue and Z represents a dibasic acid residue are also considered to be complex esters. The complex esters often have 30 to 50 carbon atoms. Polyesters, or "polyester bright stocks" can be prepared by direct esterification of dibasic acids with glycols in about equimolar quantities. The polyesterification reaction is usually continued until the product has a kinematic viscosity from about 15 to 200 centistokes at 210° F., and preferably 40 to 130 centistokes at 210° F.

Although each of these products in itself is useful as a lubricant, they are particularly useful when added or blended with each other in synthetic lubricant compositions. These esters and blends have been found to be especially adaptable to the conditions to which turbine engines are exposed, since they can be formulated to give a desirable combination of high flash point, low pour point, and high viscosity at elevated temperatures, and need contain no additives which might leave a residue upon volatilization. In addition, many complex esters have shown good stability to shear. Natural esters, such as castor oil may also be included in the blend as may be up to about 1 percent or more by weight of a foam inhibitor such as a methyl silicone polymer or other additives to provide a particular characteristic, for instance, extreme pressure or load carrying agents, corrosion inhibitors, etc., can be added.

Typical synthetic lubricants may be formulated essentially from a major amount (about 60-85%) of a complex ester and a minor amount (about 15-40%) of a diester, by stirring together a quantity of diester and complex ester at an elevated temperature, altering the proportions of each component until the desired viscosity is reached. Polyesters can be employed to thicken diester base stocks to increase the load carrying capacity of the base diester oil. The polyester will generally not comprise more than about 50 weight percent of the blend, preferably about 20 to 35 weight percent. Usually the amount of the polyester employed in any blend would be at least about 3 percent, and the majority of the lubricant is a diester. Other polymers such as acryloids may be added as thickeners to the esters, generally the single esters such as the above diesters, to obtain a base oil of desired viscosity. The acryloids are polymers of mixed C<sub>4</sub> to C<sub>18</sub> esters of methacrylic acid having 10,000 to 20,000 molecular weight. Advantageously the final lubricating oil composition would have a maximum viscosity at -40° F. of about 13,000 centistokes and a minimum viscosity of about 7.5 centistokes at 210° F.

The monohydric alcohols employed in these esters usually contain less than about 20 carbon atoms and are generally aliphatic. Preferably the alcohol contains up to about 12 carbon atoms. Useful aliphatic alcohols include butyl, hexyl, methyl, iso-octyl, and dodecyl alcohols, C<sub>13</sub> oxo alcohols and octadecyl alcohols. C<sub>8</sub> to C<sub>10</sub> branched chain primary alcohols are frequently used to improve the low temperature viscosity of the finished lubricant composition. Alcohols such as n-decanol, 2-ethylhexanol, "oxo" alcohols, prepared by the reaction of carbon monoxide and hydrogen upon the olefins obtainable from petroleum products such as diisobutylene and C<sub>7</sub> olefins, ether alcohols such as butyl carbitol, tripropylene glycol mono-isopropyl ether, di-propylene glycol mono-isopropyl ether, and products such as "Tergitol 3A3," which has the formula



are suitable alcohols for use to produce the desired lubricant. If the alcohol has no hydrogens on the beta carbon atoms, it is neo-structured; and esters of such alcohols are often preferred. In particular, the neo-C<sub>8</sub> alcohol—2,2,4-trimethyl-pentanol-1—gives lubricating diesters or complex esters suitable for blending with diesters to produce lubricants which meet stringent viscosity requirements. Iso-octanol and iso-decanol are alcohol mixtures made by the oxo process from C<sub>3</sub>-C<sub>4</sub> copolymer heptenes. The cut which makes up iso-octanol usually contains about 17% 3,4-dimethylhexanol; 29% 3,5-dimethylhexanol; 25% 4,5-dimethylhexanol; 1.4% 5,5-dimethylhexanol; 16% of a mixture of 3-methylheptanol and 5-ethylheptanol; 2.3% 4-ethylhexanol; 4.3%  $\alpha$ -alkyl alkanols and 5% other materials.

Generally, the glycols contain from about 4 to 12 carbon atoms; however, if desired they could contain a greater number. Among the specific glycols which can be employed are 2-ethyl-1,3-hexanediol, 2-propyl-3,3-heptanediol, 2-methyl-1,3-pentanediol, 2-butyl-1,3-butanediol, 2,4-diphenyl-1,3-butanediol, and 2,4-dimesityl-1,3-butanediol. In addition to these glycols, ether glycols may be used, for instance, where the alkylene radical contains 2 to 4 carbon atoms such as diethylene glycol, dipropylene glycol and other glycols up to 1000 to 2000 molecular weight. The most popular glycols for the manufacture of ester lubricants appear to be poly-propylene glycols having a molecular weight of about 100-300 and 2-ethyl hexanediol. The 2,2-dimethyl glycols, such as neopentyl glycol have been shown to impart heat stability to the final blends. Minor amounts of other glycols or other materials can be present as long as the desired properties of the product are not unduly deleteriously affected.

Aside from glycols, the esters may be made from poly-

5 hydric alcohols of more than two hydroxyl groups, e.g. tri- and tetrahydroxy aliphatic alcohols having about 4 to 12 carbon atoms preferably about 5 to 8 carbon atoms, for instance pentaerythritol, trimethylolpropane and the like. Particularly suitable ester base oils are formed when these alcohols are reacted with monocarboxylic acids having about 4 to 12 carbon atoms, preferably 4 to 9 carbon atoms. It is preferred that the reaction be conducted so as to substantially completely esterify the acids.

10 One group of monocarboxylic acids includes those of 8 to 24 carbon atoms such as stearic, lauric, etc. The carboxylic acids employed in making ester lubricants will often contain from about 4 to 12 carbon atoms. Suitable acids are described in U.S. Patent No. 2,575,195, and include the aliphatic dibasic acids of branched or straight chain structures which are saturated or unsaturated. The preferred acids are the saturated aliphatic carboxylic acids containing not more than about 12 carbon atoms, and mixtures of these acids. Such acids include 15 succinic, adipic, suberic, azelaic, and sebacic acids and "isosebacic" acid which is a mixture of  $\alpha$ -ethyl suberic acid,  $\alpha, \alpha'$ -diethyl adipic acid and sebacic acid. This composite of acids is attractive from the viewpoint of economy and availability since it is made from petroleum hydrocarbons rather than the natural oils and fats which are used in the manufacture of many other dicarboxylic acids, which natural oils and fats are frequently in short supply. The preferred dibasic acids are sebacic and azelaic or mixtures thereof. Minor amounts of adipic used with 20 a major amount of sebacic may also be used with advantage.

25 Various useful ester base oils are disclosed in United States Patents Nos. 2,499,983, 2,499,984, 2,575,195, 2,575,196, 2,703,811, 2,705,724 and 2,723,286. Generally, the synthetic base oils consist essentially of carbon, hydrogen and oxygen, i.e. the essential nuclear chemical structure is formed by these elements alone. However, these oils may be substituted with other elements such as halogens, e.g. chlorine and fluorine. Some representative components of ester lubricants are ethyl palmitate, ethyl stearate, di-(2-ethylhexyl) sebacate, ethylene glycol di-laurate, di-(2-ethylhexyl) phthalate, di-(1,3-methyl butyl) adipate, di-(2-ethyl butyl) adipate, di-(1-ethyl propyl) adipate, diethyl oxylate, glycerol tri-n-octoate, di-cyclohexyl adipate, di-(undecyl) sebacate, tetraethylene glycol-di-(2-ethylene hexoate), dicellosolve phthalate, butyl phthalyl butyl glycolate, di-n-hexyl fumarate polymer, dibenzyl sebacate, and diethylene glycol bis (2-n-butoxy ethyl carbonate). 2-ethylhexyl-adipate-neopentyl glycol-adipate-2-ethylhexyl, is a representative complex ester. Generally, these synthetic ester lubricants have a viscosity ranging from light to heavy oils, e.g. about 50 SUS at 100° F. to 250 SUS at 210° F., and preferably 30 to 150 SUS at 210° F.

55 The esters are manufactured, in general, by mere reaction of the alcoholic and acidic constituents, although simple esters may be converted to longer chain components by transesterification. The constituents, in the proportions suitable for giving the desired ester, are reacted preferably in the presence of a catalyst and solvent or water entraining agent to insure maintenance of the liquid state during the reaction. Aromatic hydrocarbons such as xylene or toluene have proven satisfactory as solvents. The choice of solvent influences the choice of temperature at which the esterification is conducted; for instance, when toluene is used, a temperature of 140° C. is recommended with xylene, temperatures up to about 195° C. may be used. To provide a better reaction rate an acid esterification catalyst is often used. 60 Many of these catalysts are known and include, for instance, HCl, H<sub>2</sub>SO<sub>4</sub>, NaHSO<sub>4</sub>, aliphatic and aromatic sulfonic acids, phosphoric acid, hydrobromic acid, HF and dihydroxy fluoboric acid. Other catalysts are thionyl chloride, boron trifluoride, and silicon tetrafluoride.

Titanium esters also make valuable esterification and transesterification catalysts.

In a preferred reaction, about 0.5 to about 1 weight percent, or advantageously, 0.2 to 0.5% of the catalyst is used with a xylene solvent at a temperature of 165 to 200° C. while refluxing water. The temperatures of the reaction must be sufficient to remove the water from the esterification mass as it is formed. This temperature is usually at least about 140° C. but not so high as to decompose the wanted product. The highest temperature needed for the reaction will probably be about 200° C., preferably not over about 175° C. The pressure is conveniently about atmospheric. Although reduced pressure or superatmospheric pressure could be utilized, there is usually no necessity to use reduced pressures, as the temperatures required at atmospheric pressure to remove the water formed do not usually unduly degrade the product.

When reacting glycols with dibasic acids to produce a polyester, it is preferred to continue the reaction with concomitant boiling off of water from the reaction mixture until the polyester product has a kinematic viscosity of about 15 to 200 centistokes at 210° F., preferably about 40 to 130 centistokes. When this point has been reached, the polymerization can be stopped, for instance, by adding a "capping alcohol" to the reaction mixture, and continuing to reflux until water ceases to be evolved. The capping alcohol is a low molecular weight mono-alcohol of up to about 20 carbon atoms. It is standard practice, when esters are made using the conventional acid catalysts such as sodium bisulfate or paratoluene-sulfonic acid to give the esters an after-treat by washing the ester with a 5 percent aqueous  $K_2CO_3$  solution or by heating the ester in an autoclave for 15 hours at 340 to 350° F. with 10 weight percent of propylene oxide. It is also conventional to subject the ester to filtration to remove insoluble materials. After this the product may be subjected to a reduced pressure distillation or stripping at 100° to 200° C. to remove volatile materials, such as water, the solvent, and light ends.

Samples of ester fluids without an oxidation inhibitor and samples containing phenothiazine alone, 5-ethyl-10,10-diphenylphenazasiline alone, phenothiazine and 2-aminopyridine and samples made according to the present invention were subjected to oxygen absorption tests. The tests were conducted at 450° F. by passing a stream of oxygen at the rate of 1 cubic foot per hour through 75 grams of the ester fluid containing the inhibitors and comparing the amount of oxygen absorbed vs. time. The induction period is signalled by a marked increase of oxygen absorption. The results of these tests are shown in Table I.

The lengths of the induction periods serve as a significant measure of the relative effectiveness of the inhibitors. As shown in Table I addition of the novel additive combination of the present invention protects the fluid against rapid oxidation for a longer period of time than would be expected if the effect were simply additive.

Other examples of formulations made in accordance with the present invention are as follows:

|    | EXAMPLE I                           | Parts by wt. |
|----|-------------------------------------|--------------|
| 10 | Plexol-201 <sup>1</sup>             | 97.5         |
|    | Titanium polymer <sup>2</sup>       | 1.0          |
|    | Phenothiazine                       | 0.5          |
| 15 | 5-ethyl-10,10-diphenylphenazasiline | 1.0          |
|    | 2-aminopyridine                     | 0.5          |
|    | D.C.F. 200-60,000 <sup>3</sup>      | 0.001        |

<sup>1</sup> A diethylhexyl sebacate oil having a kinematic viscosity of 100° F. of 12.3 cs., a viscosity index of 154, a pour point of below -80° F. and acid No. of 0.12.

<sup>2</sup> A polymer derived from tetrabutyl titanate and 2-ethyl-1,3 hexanediol.

<sup>3</sup> D.C.F. 200-60,000 is a methyl silicone polymer having a viscosity of 60,000 cs. at 25° C. and is an anti-foaming agent.

|    | EXAMPLE II                          | Parts by wt. |
|----|-------------------------------------|--------------|
| 25 | Plexol-255 <sup>1</sup>             | 98.75        |
|    | Phenothiazine                       | 0.5          |
|    | Glycol titanate <sup>2</sup>        | 0.25         |
|    | 5-ethyl-10,10-diphenylphenazasiline | 1.0          |
|    | 2-aminopyridine                     | 0.5          |
| 30 | Sebacic acid                        | .0075        |
|    | D.C.F. 200-60,000                   | .001         |

<sup>1</sup> A mixture of diisooctyl adipate, ditridecyl sebacate, and Acryloid-966 (a copolymer of alkyl with acrylates and N-vinyl pyrrolidone).

<sup>2</sup> Polymer of titanium tetra-alkyl esters and glycol.

|    | EXAMPLE III                         | Parts by wt. |
|----|-------------------------------------|--------------|
|    | Diisooctyl azelate                  | 25.5         |
| 40 | Complex ester <sup>1</sup>          | 74.0         |
|    | Phenothiazine                       | 0.5          |
|    | Free azelaic acid                   | 0.01         |
|    | 5-ethyl-10,10-diphenylphenazasiline | 1.0          |
|    | 2-aminopyridine                     | 0.5          |
| 45 | D.C.F. 200-60,000                   | 0.001        |

<sup>1</sup> Derived from the reaction of one mole of neopentyl glycol,

2 moles of azelaic acid and two moles of isoctyl alcohol.

In the compositions of Table I and of Examples I, II, and III, the 2-aminopyridine can be replaced with 0.5 parts by weight of 3-aminoquinoline and obtain essentially the same results.

TABLE I

## Results of Oxygen Absorption Tests

[Conditions: 450° F.; 1 ft.<sup>3</sup> O<sub>2</sub>/hr.; 75 g. fluid]

| Run No. | Base fluid         | Additives                                         | Conc. (wt. percent) | Induction period (min.) | Total time (min.) | Volume O <sub>2</sub> absorbed (ml.) |
|---------|--------------------|---------------------------------------------------|---------------------|-------------------------|-------------------|--------------------------------------|
| 80      | Oil A <sup>1</sup> | None                                              |                     | 5                       | 119               | 3,000                                |
| 129     | do <sup>1</sup>    | Phenothiazine                                     | 0.5                 | 117                     | 146               | 2,500                                |
| 130     | do <sup>1</sup>    | do                                                | 1.0                 | 205                     | 247               | 2,500                                |
| 263     | do <sup>1</sup>    | { Phenothiazine<br>2-aminopyridine                | 0.5<br>0.5          | 305                     | 361               | 2,500                                |
| 313     | do <sup>1</sup>    | { Phenothiazine<br>2-aminopyridine                | 0.5<br>0.5          |                         | 2468              | 925                                  |
| 168     | do <sup>1</sup>    | 2-ethyl-10,10-diphenylphenazasiline               | 1.0                 | 5                       | 47                | 2,500                                |
| 304     | do <sup>1</sup>    | Phenothiazine 5-ethyl-10,10-diphenylphenazasiline | { 0.5<br>1.0        | 319                     | 388               | 2,500                                |

<sup>1</sup> An ester from pentaerythritol and a mixture of aliphatic acids with an average chain length of seven carbons.

<sup>2</sup> The test was stopped at this point. The end of the induction period had not been reached, however.

We claim:

1. A lubricant composition consisting essentially of an ester-based fluid of lubricating viscosity and minor amounts effective to retard oxidation of said ester-based fluid at temperatures in excess of 400° F., of about .01 to 5 percent by weight of phenothiazine, about .01 to 5 percent by weight of 5-alkyl-10,10-diphenylphenazasiline wherein the alkyl group contains 1 to 4 carbon atoms, and about .01 to 5 percent by weight of a compound selected from the group consisting of aminoquinoline and aminopyridine, said ester-based fluid being an ester of an alkanol of 4-10 carbon atoms and an alkane carboxylic acid of 4-12 carbon atoms.

2. The composition of claim 1 wherein the compound selected is aminopyridine.

3. The composition of claim 1 wherein the compound selected is aminoquinoline.

4. The lubricant composition of claim 1 containing about 0.1 to 2 percent by weight of phenothiazine, about 0.1 to 2 percent by weight of 5-ethyl-10,10-diphenylphenazasiline and about 0.1 to 2 percent by weight of a

material selected from the group consisting of 2-amino-pyridine and 3-aminoquinoline.

References Cited in the file of this patent

UNITED STATES PATENTS

|           |                   |       |               |
|-----------|-------------------|-------|---------------|
| 2,216,711 | Musher            | ----- | Oct. 1, 1940  |
| 2,318,196 | Chenicek          | ----- | May 4, 1943   |
| 2,950,250 | Fainman           | ----- | Aug. 23, 1960 |
| 3,036,005 | Kock              | ----- | May 22, 1962  |
| 3,038,858 | Verley            | ----- | June 12, 1962 |
| 3,038,859 | Eickemeyer et al. | ----- | June 12, 1962 |

OTHER REFERENCES

Cohen et al.: "Aliphatic Esters," I. and E. Chem., vol. 45, No. 8, August 1953, pages 1766-1775.

Dintses et al.: "Synthetic Lubricating Oils," pub. by Liaison Offices, Technical Information Center, Wright Patterson AFB, Ohio, F-TS-9719, August 1959, pages 283-304.

Rodd: Chemistry of Carbon Compounds, vol. IVc (1960), page 1519, QD, 251, R6.